

## 1

3,310,399

## ALLOYS FOR USE AT HIGH TEMPERATURES

James French Baldwin, 78 Forest Ave.,  
Locust Valley, N.Y. 11560  
No Drawing. Filed July 10, 1964, Ser. No. 381,932  
9 Claims. (Cl. 75—171)

The present invention relates to nickel base alloys which consist essentially of nickel with substantial proportions of chromium, molybdenum, tantalum, cobalt, titanium and aluminum, which are highly corrosion and erosion resistant at the temperatures encountered in gas turbines and jet engines, in the range of 1700° F. to 2200° F. and have relatively great tensile strength at operating temperatures, as well as the required degree of elongation and creep.

The higher the temperature at which a blade or vane in a gas turbine engine can be operated the higher the efficiency of the engine, and it is likewise obvious that the blades and vanes should have a relatively long life at the temperature at which they are to be operated. The alloys of the present invention are particularly suited to fulfilling all of the requirements of a blade or vane for gas turbine engines at higher than conventional temperatures and this is shown by the ability of the blades and vanes formed from alloys of the present invention to withstand exceedingly high operating temperatures for short periods of time, or to withstand higher than normal operating temperatures for extended periods of time, depending upon whether the engine is intended for military or commercial use.

Among the alloys of the prior art which are currently used are those disclosed in the United States Patents Nos. 2,948,606, 3,005,704 and 3,061,426, as well as 3,026,198.

Patent No. 2,948,606 requires a relatively large amount of tungsten and is suitable for use only to a maximum temperature of 2000° F., and generally at a much lower temperature, such as 1800° F.

Patent No. 3,005,704 is differentiated from the alloys of the present invention in that it includes no cobalt content in its alloys, and is capable of operating up to a maximum of about 1900° F.

Patent No. 3,026,198 discloses alloys which require from 20 to 35% of tungsten, and which differ in many other respects from the alloys of the present invention. Furthermore the alloys disclosed in this patent do not have the properties required for extended operation at temperatures in excess of 2000° F.

Patent No. 3,061,426 discloses other alloys which have different ratios of the titanium and aluminum content than the alloys of the present invention, and further require the use of substantial amounts of vanadium which are detrimental in the alloys of the present invention. Additionally, the alloys of this patent require no tantalum content, and are adapted for use only at temperatures of the order of 1700° F. Whereas, alloys according to this patent have a density of 0.308 pound per cubic inch, alloys of the present invention have a density as low as 0.297 pound per cubic inch. Alloys of the present invention generally have an incipient melting point from 20° to 25° F. above an alloy of this patent, later referred to herein as alloy #100.

The alloys of the present invention are characterized by their ability to operate at temperatures in the range of 1700° F. to 2200° F. for relatively long and acceptable periods of time, with adequate strength and other properties so that they may be used as the alloy to form the blades of an extremely efficient gas turbine engine.

The present invention has for its object the provision of novel and improved high-temperature, corrosion and erosion resistant alloys which are able to withstand prolonged operation at temperatures of about 2000° F. and

## 2

higher, and which have relatively long life under operating conditions at these temperatures.

The present invention has for another object the provision of novel and improved high-temperature alloys of the class described which are capable of being cast with relatively consistent results, as distinguished from many prior art alloys which give erratic results, depending upon minute variations in the many variables in the casting process.

10 The alloys of the present invention also have relatively high incipient melting temperatures so that they may be heat-treated at higher than normal temperatures and may be operated at temperatures above ordinary operating temperatures with no danger of the blades being weakened by incipient melting.

15 The alloys of the present invention show a remarkable combination of strength and ductility at high temperature levels, and are superior to most of those of the prior art, combining these properties with other properties to an unusually high degree. Additionally, these alloys of the present invention show an unusually high thermal shock resistance which is much better than that of other high strength alloys.

20 25 Further, alloys of the present invention are less susceptible to bowing when used as stator vanes in jet turbine engines than conventional nickel and cobalt base alloys now used for that purpose.

20 25 30 Moreover, the alloys of the present invention do not develop a sigma phase after exposure for long periods of time, such as 1000 to 4000 hours at temperatures in the neighborhood of 1500° to 1650° F., as is common with other nickel base alloys of generally similar strength.

30 35 40 Additionally, alloys of this invention can be successfully extruded, upset and forged, while conventional nickel base alloys, such as are used for jet turbine blades and vanes, generally are not susceptible to such operations, and in the few cases where such conventional alloys have been extruded, upset or forged, it has been accomplished with only extreme difficulty.

40 45 50 The alloys of the present invention respond readily to heat treatment and show solution temperatures as high as 2300° F., and their ready response to aging imparts great stability for long periods of use and restores strength and ductility after exposure to temperature in the region of 2000° F., such as are used in the coating of blades and vanes.

50 55 60 The alloys of this invention by weight consist essentially of from 5.0% to 12.0% chromium, about 3.0% to 8.0% molybdenum, 2.3% to 10.0% tantalum, 5.0% to 15.5% cobalt, 0 to 7.0% titanium, 0.0% to 8.0% aluminum, up to 0.25% carbon, up to .050% boron, with zirconium up to 1.0%, balance essentially nickel in a quantity of at least 45%. In these alloys, the combined content of the molybdenum and tantalum varies from 5% to 14%, and the combined content of titanium and aluminum varies from 5% to 8.8%. It is preferable to hold manganese and silicon to a maximum of 1.0%, iron to not more than 5.0%, with a low content of phosphorus of about 0.02% maximum and sulphur about 0.02% maximum. Deoxidizers, such as calcium, magnesium and rare earths can be used in the usual small quantities in the preparation of the alloys.

65 70 75 Within the broader composition ranges of the present invention, there are narrower ranges which yield the preferred alloy compositions of the present invention, one group comprising higher ranges of chromium content with a relatively high molybdenum content and a relatively low cobalt content, while another group includes alloys having lower ranges of chromium content with lower ranges of molybdenum and higher ranges of cobalt.

Of these two groups, the first is preferred including

from 7.5% to 12% by weight of chromium, from 3.0% to 8.0% of molybdenum, about 10% (5.0% to 10.5%) of cobalt, from 2.3% to 10.0% of tantalum, up to 2.5% of titanium and from 5.0% to 7.0% aluminum.

The second group includes alloys which include from 5% to 8% of chromium, from 3% to 6% of molybdenum, from 4% to 8% of tantalum, from 1% to 2.3% titanium and from 4.0% to 8.0% of aluminum, and from 10% to 15.5% of cobalt, preferably from 13.0% to 15.5%.

Such alloys will have compositions within the following broad range and one or the other of the following narrower ranges.

|                      | Percent by wt. |
|----------------------|----------------|
| Mo + Ta              | 9.75-10.75     |
| Cobalt               | 9.50-10.50     |
| Titanium             | 0.80-1.20      |
| 5 Aluminum           | 5.75-6.25      |
| Ti + Al              | 6.55-7.45      |
| Boron                | 0.01-0.02      |
| Zirconium            | 0.05-0.10      |
| Manganese, (maximum) | 0.10           |
| Iron, (maximum)      | 0.25           |
| Sulfur, (maximum)    | 0.015          |
| Silicon, (maximum)   | 0.40           |

|                         | Broadest Range | Broad Range | Group A    | Group B    |
|-------------------------|----------------|-------------|------------|------------|
| Carbon                  | 0.3% max.      | 0.3% max.   | 0.3% max.  | 0.3 max.   |
| Chromium                | 5-12%          | 5-12%       | 7.5-12%    | 5-8%       |
| Molybdenum              | 3-8.0%         | 3-8.0%      | 3-8.0%     | 3-6%       |
| Tantalum                | 2.3-10%        | 2.3-10%     | 2.3-10%    | 4-8%       |
| Molybdenum and tantalum | 5-14%          | 5-14%       | 7-13%      | 7-12.2%    |
| Cobalt                  | 5-15.5%        | 5-15.5%     | 5-10.5%    | 10-15.5%   |
| Titanium                | 0-7%           | 2.5% max.   | Up to 2.5% | 1-2.3%     |
| Aluminum                | 0-7%           | 4.0-8.0%    | 5-7%       | 4-8%       |
| Titanium and aluminum   | 5-8.8%         | 5-8.8%      | 5.5-8.0%   | 5.4-8.8%   |
| Boron                   | 0.05% max.     | 0.05% max.  | 0.05% max. | 0.05% max. |
| Zirconium               | 1.0% max.      | 1.0% max.   | 1.0% max.  | 1.0% max.  |
| Iron                    | 2% max.        | 2% max.     | 2% max.    | 2% max.    |
| Vanadium                | 0%             | 0%          | 0%         | 0%         |
| Tungsten                | 2.5% max.      | 2.5% max.   | 2.5% max.  | 2.5% max.  |
| Phosphorous             | 0.02% max.     | 0.02% max.  | 0.02% max. | 0.02% max. |
| Sulfur                  | 0.02% max.     | 0.02% max.  | 0.02% max. | 0.02% max. |
| Nickel                  | Balance        | Balance     | Balance    | Balance    |

The balance of the alloys is essentially nickel, but may include trivial or trace amounts of various impurities such as the following elements in amounts of substantially the following weight percentages as maximum amounts for each of the several elements:

|                                    | Percent |
|------------------------------------|---------|
| Manganese (preferably about 0.10%) | 0.20    |
| Iron (preferably about 0.30%)      | 2.0     |
| Sulfur (preferably about 0.015%)   | 0.20    |

|                        |      |
|------------------------|------|
| Columbium, (maximum)   | 0.10 |
| Phosphorus, (maximum)  | 0.20 |
| Vanadium               | 0    |
| 35 Tungsten, (maximum) | 0.10 |
| Nickel, remainder.     |      |

Some of the alloys of the prior art most commonly used in gas turbines have specification analyses, as follows, hereinafter referred to as alloys 100, 101 and 102.

|                         | #100        | #101        | #102          |
|-------------------------|-------------|-------------|---------------|
| Carbon                  | 0.15-0.2%   | 0.12-0.17%  | 0.20% max.    |
| Manganese               | 0.20% max.  | 0.20% max.  | 1.00 max.     |
| Sulfur                  | 0.015% max. | 0.015% max. | 0.015 max.    |
| Silicon                 | 0.20% max.  | 0.20% max.  | 1.00 max.     |
| Chromium                | 8.0-11.0%   | 8.0-10.0%   | 13.00-15.00.  |
| Molybdenum              | 2.0-4.0%    |             | 3.50-5.50.    |
| Columbium               |             | 0.75-1.25%  |               |
| Columbium plus Tantalum |             |             | 1.00-3.00.    |
| Molybdenum and Tantalum |             |             | 4.50-8.50.    |
| Titanium                | 4.5-5.5%    | 1.75-2.25%  | 0.75-1.25.    |
| Aluminum                | 5.0-6.0%    | 4.75-3.25%  | 5.50-6.50.    |
| Titanium and Aluminum   | 10.0-11.5%  |             | 6.25-7.75.    |
| Tungsten                |             | 11.5-13.5%  |               |
| Boron                   | 0.01-0.02%  | 0.1-0.2%    | 0.0005-0.015. |
| Zirconium               | 0.03-0.09%  | 0.03-0.08%  | 0.05-0.12.    |
| Iron                    | 1.0% max.   | 1.5% max.   | 3.00 max.     |
| Copper                  |             | 0.10% max.  | 0.50 max.     |
| Cobalt                  | 13.0-17.0%  | 9.0-11.0%   | 1.00 max.     |
| Vanadium                | 0.70-1.2%   | Remainder   | 1.00 max.     |
| Nickel                  |             | Remainder   | Remainder.    |

|                       |      |
|-----------------------|------|
| Silicon, maximum      | 0.40 |
| Columbium, maximum    | 0.20 |
| Phosphorus, maximum   | 0.02 |
| Vanadium, trace only. |      |

The more specific and preferred composition range for the alloys of my present invention are as follows:

|            | Percent by wt. |
|------------|----------------|
| Carbon     | 0.08-0.13      |
| Chromium   | 7.50-8.50      |
| Molybdenum | 5.75-6.25      |
| Tantalum   | 4.00-4.50      |

It may be noted that alloys #100 and #102 are of the usual run of chromium, molybdenum, titanium, aluminum and cobalt, with alloy #101 substituting tungsten for molybdenum. Alloy #100 includes an essential vanadium content with no tantalum. In alloys #100 and #101 tantalum is not used and in alloy #102 its presence with 65 columbium is incidental as an impurity in the columbium, and tantalum is not an essential element in alloy #102.

Typical and preferred examples of alloys according to the present invention have the following compositions, expressed in percent by weight, the properties of which 70 alloys will be set forth below.

## WEIGHT PERCENT OF ALLOY CONSTITUENTS

|                      | Example |         |         |         |         |
|----------------------|---------|---------|---------|---------|---------|
|                      | No. 1   | No. 2   | No. 3   | No. 4   | No. 5   |
| Carbon               | 0.09    | 0.07    | 0.10    | 0.07    | 0.06    |
| Chromium             | 7.8     | 7.7     | 7.9     | 7.8     | 7.7     |
| Molybdenum           | 5.8     | 4.0     | 3.95    | 5.8     | 6.2     |
| Tantalum             | 2.3     | 7.98    | 7.5     | 6.2     | 4.4     |
| Mo plus Ta           | 8.1     | 9.0     | 11.8    | 12.0    | 10.6    |
| Cobalt               | 10.1    | 9.75    | 9.9     | 9.9     | 10.0    |
| Titanium             | 2.3     | 1.1     | 1.0     | 2.1     | 1.1     |
| Aluminum             | 6.0     | 6.2     | 5.9     | 5.9     | 6.3     |
| Ti plus Al           | 8.3     | 7.3     | 6.9     | 8.0     | 7.4     |
| Boron                | 0.018   | 0.012   | 0.012   | 0.024   | 0.012   |
| Zirconium            | 0.08    | 0.1     | 0.09    | 0.07    | 0.1     |
| Nickel (essentially) | Balance | Balance | Balance | Balance | Balance |

The alloy of Example No. 1 had the following mechanical properties:

Standard tensile strength test specimens at room temperature showed an ultimate tensile strength of 137,000 p.s.i., with 6% elongation and 8.4% reduction in area; and a yield strength with 0.2% elongation of 121,000 p.s.i.

At 1800° F. and a loading of 85,000 p.s.i., specimens ruptured after 26.2 hours, showing an elongation of 2% after rupture and an area reduction of 6.0%. When tested at 1800° F. and a loading of 29,000 p.s.i., the specimens ruptured after 23.0 hours, with 2.5% elongation after rupture and 2.2% area reduction.

At 1900° F. with 18,000 p.s.i. loading the test bar ruptured after 32.1 hours with 2.4% elongation and 2.0% reduction in area.

The alloy of Example No. 2 had the following mechanical properties:

At 1800° F. tensile strength specimens of the cast alloy

000 p.s.i. rupture occurred at 111.3 hours with 8.3% elongation and 4.9% reduction. When tested at 2000° F. and a loading of 18,000 p.s.i., the specimens ruptured after 63.4 hours, with 3.0% elongation after rupture and 2.1% area reduction.

Another specimen of the alloy of Example No. 3 had the following mechanical properties:

Standard tensile strength test specimens at room temperature showed an ultimate tensile strength of 138,000 p.s.i., with 6.0% elongation and 11.5% reduction in area and a yield strength with 0.2% elongation of 114,250 p.s.i.

Similar test specimens cast from the same heat showed the following properties on rupture, the column headings indicating temperature, continuously applied axial stress in pounds per square inch, hours a rupture, percentage elongation and percentage reduction in area, hours, and percentage extension prior to rupture.

| Temp., ° F. | P.s.i.  | Hours | El., percent | Percent R.A. | Hours | Percent Ext. |
|-------------|---------|-------|--------------|--------------|-------|--------------|
| 1,400       | 100,000 | 32.3  | 3.2          | 6.2          | 29.6  | 1.651        |
| 1,400       | 94,000  | 102.3 | 2.4          | -----        | ----- | 1.46         |
| 1,400       | 85,000  | 298.4 | 3.0          | -----        | ----- | 1.46         |
| 1,800       | 29,000  | 70.8  | 8.5          | -----        | ----- | -----        |
| 1,850       | 29,000  | 17.3  | 7.5          | 7.3          | 15.4  | 3.134        |
| 1,900       | 18,000  | 91.4  | 9.0          | -----        | ----- | -----        |
| 2,000       | 10,000  | 172.6 | 9.6          | 11.4         | 171.9 | 4.434        |

maintained under continuously applied axial stress of 29,000 p.s.i. ruptured after 22.2 hours, and exhibited an elongation after rupture of 2.0%, and an area reduction

Long time creep and rupture tests on test specimens from virgin melts having substantially the same analysis as Example 3 gave the following results:

| Temperature                    | 1,500° F. | 1,500° F. | 1,500° F. | 1,500° F. | 1,700° F. | 1,750° F. | 1,800° F. | 1,950° F. |
|--------------------------------|-----------|-----------|-----------|-----------|-----------|-----------|-----------|-----------|
| P.s.i.                         | 60,000    | 55,000    | 50,000    | 40,000    | 25,000    | 21,000    | 15,000    | 8,000     |
| Prior extension (hrs.)         | 360.9     | 1,933.0   | 4,567.0   | 4,532.7+  | 1,413.7   | 1,066.1   | 1,930.0   | 1,253.8   |
| Prior extension creep, percent | 1.038     | 4.481     | 3.964     | 0.415     | 6.930     | 8.048     | 10.015    | 6.105     |
| Final elongation, percent      | (1)       | 5.7       | 4.9       | -----     | 8.4       | 10.1      | 10.7      | 9.5       |
| Reduction in area, percent     |           | 7.8       | 6.3       | -----     | 13.5      | 13.9      | 11.2      | 19.0      |

<sup>1</sup> Stopped at 1%.

of 1.0%. At 1900° F. and a loading of 18,000 p.s.i., specimens ruptured after 63.4 hours, showing an elongation of 3.0% after rupture and an area reduction of 2.1%.

The alloy of Example No. 3 had the following mechanical properties:

Standard tensile strength test specimens at room temperature showed a tensile strength of 161,000 p.s.i. with 10.0% elongation and 11.0% reduction in area; and a yield strength with 0.2% elongation of 141,000 p.s.i.

At 1400° F. a tensile strength specimen of the cast alloy maintained under continuously applied axial stress of 85,000 p.s.i. ruptured after 367.4 hours, and exhibited an elongation after rupture of 4.7%, and an area reduction of 4.7%. At 1600° F. and 55,000 p.s.i. the specimen ruptured at 105.1 hours with 4.6% elongation and 4.1% reduction. At 1700° F. with 40,000 p.s.i. loading, the specimen ruptured at 71.6 hours with 5.3% elongation and 4.8% reduction. At 2000° F. with 10,-

60 The alloy of Example No. 4 had the following mechanical properties:

Standard tensile strength test specimens at room temperature showed an ultimate tensile strength of 145,000 p.s.i., and a yield strength with 0.2% elongation of 119,000 p.s.i.

At 1400° F. tensile strength specimens of the cast alloy maintained under continuously applied axial stress of 85,000 p.s.i. ruptured after 166.9 hours, and exhibited an elongation after rupture of 3.0%, and an area reduction of 5.0%. At 1800° F. and a loading of 29,000 p.s.i., specimens ruptured after 32.0 hours, showing an elongation of 4.5% after rupture and an area reduction of 3.1%. When tested at 1900° F. and a loading of 18,000 p.s.i. the specimens ruptured after 53.0 hours, with 2.0% elongation after rupture and 8.0% area reduction.

The alloy of Example No. 5 had the following mechanical properties:

Standard tensile strength test specimens at room temperature showed a tensile strength of 140,000 p.s.i., with 5.0% elongation and 8.0% reduction in area, and a yield strength with 0.2% elongation of 125,000 p.s.i.

At 1800° F. and a loading of 29,000 p.s.i., specimens ruptured after 14.1 hours, showing an elongation of 3.1% after rupture and an area reduction of 4.6%. When tested at 1900° F. and a loading of 18,000 p.s.i., the specimens ruptured after 41.4 hours, with 4.0% elongation after rupture and 4.7% area reduction.

#### WEIGHT PERCENT OF ALLOY CONSTITUENTS

|            | Example |         |         |         |         |
|------------|---------|---------|---------|---------|---------|
|            | No. 6   | No. 7   | No. 8   | No. 9   | No. 10  |
| Carbon     | 0.09    | 0.1     | 0.1     | 0.1     | 0.1     |
| Chromium   | 8.0     | 8.0     | 8.1     | 8.1     | 8.1     |
| Molybdenum | 5.8     | 5.9     | 6.1     | 6.0     | 6.2     |
| Tantalum   | 4.3     | 4.2     | 4.2     | 4.2     | 4.4     |
| Mo+Ta      | 10.1    | 10.1    | 10.3    | 10.2    | 10.6    |
| Cobalt     | 9.8     | 10.1    | 10.0    | 9.9     | 11.8    |
| Titanium   | 1.0     | 1.0     | 1.0     | 1.0     | 1.05    |
| Aluminum   | 5.9     | 5.9     | 6.0     | 6.0     | 6.2     |
| Ti+Al      | 6.9     | 6.9     | 7.0     | 7.0     | 7.25    |
| Boron      | 0.012   | 0.013   | 0.012   | 0.012   | 0.01    |
| Zirconium  | 0.1     | 0.08    | <0.012  | 0.08    | 0.01    |
| Iron       | 0.2     | 0.2     | 0.2     | 0.2     | -----   |
| Vandium    | 0.0     | 0.0     | 0.0     | 0.0     | -----   |
| Tungsten   | <0.1    | <0.1    | <0.1    | <0.1    | -----   |
| Silicon    | 0.4     | 0.27    | 0.18    | 0.19    | -----   |
| Manganese  | <0.1    | <0.1    | <0.02   | <0.1    | -----   |
| Sulfur     | 0.005   | 0.006   | 0.008   | 0.004   | -----   |
| Columbium  | -----   | -----   | <0.1    | -----   | -----   |
| Nickel     | Balance | Balance | Balance | Balance | Balance |

The alloy of Example No. 6 had the following mechanical properties:

Standard tensile strength test specimens at room temperature showed a tensile strength of 149,000 p.s.i., with an elongation of 9.0%, and a yield strength with 0.2% elongation of 121,000 p.s.i.

At 1400° F. tensile strength specimens of the cast alloy maintained under continuously applied axial stress of 85,000 p.s.i. ruptured after 339.3 hours, and exhibited an elongation after rupture of 3.1%. At 1800° F. and a loading of 2,900 p.s.i., specimens ruptured after 52.4 hours, showing an elongation of 5.1% after rupture.

The alloy of Example No. 7 had the following mechanical properties:

| Melt                                        | Revert  | Virgin  | Duo Melt | Revert  | Virgin  | Duo Melt | Revert   | Duo      | Duo      |
|---------------------------------------------|---------|---------|----------|---------|---------|----------|----------|----------|----------|
| Temp., ° F.                                 | 1,500   | 1,500   | 1,500    | 1,500   | 1,500   | 1,500    | 1,500    | 1,500    | 1,500    |
| P.s.i.                                      | 50,000  | 50,000  | 50,000   | 45,000  | 45,000  | 45,000   | 40,000   | 40,000   | 40,000   |
| Hrs. prior ext.                             | 1,866.7 | 1,775.2 | -----    | 3,924.4 | 3,954.5 | -----    | 5,299.0+ | 4,647.6+ | 5,182.0+ |
| Prior Ext. Creep, percent                   | 1.896   | 1.586   | -----    | 5.425   | 2.612   | -----    | 479      | 917      | -----    |
| Final hrs.                                  | 1,868.0 | 1,784.9 | 2,160.8  | 3,925.0 | 3,965.0 | 3,124.5  | (1)      | (1)      | (1)      |
| Final Elong., percent                       | 2.4     | 2.2     | 6.5      | 5.6     | 3.6     | 5.0      | -----    | -----    | -----    |
| Final R.A., percent                         | 6.6     | 3.9     | 5.5      | 9.3     | 5.6     | 3.9      | -----    | -----    | -----    |
| Ultimate Tensile                            | 155,000 | 143,000 | 141,000  | -----   | -----   | -----    | -----    | -----    | -----    |
| Elongation, percent                         | 8.0     | 9.0     | 11.0     | -----   | -----   | -----    | -----    | -----    | -----    |
| 0.2% Yield                                  | 123,000 | 120,000 | 110,000  | -----   | -----   | -----    | -----    | -----    | -----    |
| Rupture, 1,400° F., 85,000 p.s.i.<br>(hrs.) | 176.6   | 88.6    | 142.6    | -----   | -----   | -----    | -----    | -----    | -----    |
| Percent Elong.                              | 4.0     | 2.0     | 4.0      | -----   | -----   | -----    | -----    | -----    | -----    |
| 1,800° F., 29,000 p.s.i. (hrs.)             | 44.9    | 35.5    | 39.8     | -----   | -----   | -----    | -----    | -----    | -----    |
| Percent Elong.                              | 4.0     | 3.0     | 5.0      | -----   | -----   | -----    | -----    | -----    | -----    |

<sup>1</sup> No Rupture.

Standard tensile strength test specimens at room temperature showed a tensile strength of 142,000 p.s.i., with an elongation of 11.0%, and a yield strength with 0.2% elongation of 112,000 p.s.i.

At 1400° F. tensile strength specimens of the cast alloy maintained under continuously applied axial stress of 85,000 p.s.i. ruptured after 205.8 hours, and exhibited an elongation after rupture of 5.0%. At 1800° F. and a loading of 29,000 p.s.i., specimens ruptured after 51.4 hours, showing an elongation of 6.0% after rupture.

After strain-aging specimens of this alloy at 1650° F. and 15,000 p.s.i. for over 1000 hours, strain-aged speci-

mens exhibited 4% room temperature ductility as compared with 7-11% for unaged specimens from the same heat and cast. Examination of the strain-aged and as cast specimens showed no evidence of the sigma phase in the strain aged specimens.

The alloy of Example No. 8 had the following mechanical properties:

Standard tensile strength test specimens at room temperature showed a tensile strength of 143,000 p.s.i., with an elongation of 8%, and a yield strength with 0.2% elongation of 118,000 p.s.i.

At 1400° F. tensile strength specimens of the cast alloy maintained under continuously applied axial stress of 85,000 p.s.i. ruptured after 134.7 hours, and exhibited an elongation after rupture of 3.7%. At 1800° F. and a loading of 29,000 p.s.i., specimens ruptured after 49.3 hours, showing an elongation of 3.5% after rupture.

Other melts of alloys approximating the composition of Examples 6, 7 and 8 had the following analyses (weight percent of alloy constituents):

| Example              | A       | B       | C       |
|----------------------|---------|---------|---------|
| Carbon               | 0.1     | 0.1     | 0.1     |
| Chromium             | 7.9     | 8.0     | 8.2     |
| Molybdenum           | 6.0     | 6.05    | 6.05    |
| Tantalum             | 4.65    | 4.30    | 4.30    |
| Mo + Ta              | 10.65   | 10.35   | 10.35   |
| Cobalt               | 9.85    | 10.0    | 9.75    |
| Titanium             | 1.0     | 0.97    | 0.98    |
| Aluminum             | 6.1     | 6.0     | 5.95    |
| Ti + Al              | 7.1     | 6.97    | 6.93    |
| Boron                | 0.012   | 0.013   | 0.013   |
| Zirconium            | 0.08    | 0.08    | 0.08    |
| Nickel (essentially) | Balance | Balance | Balance |

Trivial elements, as given for Examples 6, 7 and 8.

Tests on specimens of different melts of alloys having the analyses of Examples A, B and C gave the following properties:

| Temp., ° F. | .2% Elonga-tion | Ultimate (p.s.i.) | Percent Elong. | Percent Red. of Area |
|-------------|-----------------|-------------------|----------------|----------------------|
| 2,000       | 24,100          | 40,400            | 10.2           | 16.9                 |
| 2,000       | 26,800          | 42,100            | 8.9            | 9.8                  |
| 2,100       | 29,900          | 43,700            | 12.2           | 13.9                 |
| 2,100       | 30,100          | 44,100            | 16.1           | 15.1                 |
| 2,200       | 8,900           | 14,700            | 18.7           | 22.1                 |
| 2,200       | 8,500           | 14,100            | 17.9           | 13.7                 |

The alloy of Example No. 9 had the following mechanical properties:

Standard tensile strength test specimens at room temperature showed a tensile strength of 141,000 p.s.i., with 8.0% elongation, and a yield strength with 0.2% elongation of 119,000 p.s.i.

At 1400° F. tensile strength specimens of the cast alloy maintained under continuously applied axial stress of 85,000 p.s.i. ruptured after 140.3 hours, and exhibited an elongation after rupture of 2.7%. At 1800° F. and a loading of 29,000 p.s.i., specimens ruptured after 42.2 hours, showing 3% elongation.

The alloy of Example No. 10 had the following mechanical properties:

Standard tensile strength test specimens at room temperature showed a tensile strength of 137,000 p.s.i. with a 6.0% elongation accompanied by a 13.0% reduction in area, and a yield strength with 0.2% elongation of 126,000 p.s.i.

At 1400° F. test specimen showed an ultimate strength of 135,000 p.s.i. rupture with 3.0% elongation and 5.0% reduction in area; and a yield strength of 121,000 p.s.i. at 2% elongation.

At 1400° F. tensile strength specimens of the cast alloy maintained under continuously applied axial stress of 85,000 p.s.i. ruptured after 87.7 hours, and exhibited an elongation after rupture of 4.2%.

At 1800° F. and at a loading of 85,000 p.s.i., the specimen ruptured after 87.7 hours, showing 4.2% elongation and a reduction in area of 2.4%.

At 1900° F. and 18,000 p.s.i. rupture occurred at 33.3 hours with 6.2% elongation and 9.3% reduction in area.

Alloys similar to those of Examples 6 to 10 may be heat treated and forged to yield forgings which display greatly superior properties, as compared with the alloys of the prior art.

Tests were carried out on specimens of various heats, all falling within the following ranges:

198,000 p.s.i. (ultimate strength with 23.0% elongation and 20.0% reduction in area).

Long time creep tests of specimens of alloys falling within the narrow ranges just given above, gave the following data:

| Prior treatment                 | Temp., °F.                                  | Stress, p.s.i. | Stopped at hrs. | Percent Creep |
|---------------------------------|---------------------------------------------|----------------|-----------------|---------------|
| 10 2,000° F., 4 hours<br>Coated | 1,500                                       | 55,000         | 576.0           | 1.05          |
|                                 | 1,600                                       | 30,000         | 1,795.5         | 1.009         |
|                                 | 1,700                                       | 21,000         | 1,481.2         | 1.014         |
|                                 | 1,900                                       | 8,000          | 497.4           | 0.463         |
|                                 | 2,000                                       | 5,000          | 806.4           | 1.017         |
|                                 | 2,000 F., 4 hours, then 1,600° F., 50 hours | 1,500          | 55,000          | 436.6         |
| 15 Coated                       | 1,700                                       | 21,000         | 1,482.9         | 1.000         |
|                                 | 1,600                                       | 30,000         | 2,322.5         | 1.005         |

The coated specimens were subjected to the procedure set forth in United States Patent No. 3,102,044 using 2000° F. for 4 hours, followed by heating at 1600° F. for 50 hours, while the sixth specimen above was subjected to the same temperatures but without any coating material.

In stress-rupture tests of heat-treated specimens of alloys within this narrow range, the following data were observed:

| Heat treatment, °F., hours | Temp., °F. | Stress, p.s.i. | Rupture Time, hrs. | Percent Elong. | Percent R.A. |
|----------------------------|------------|----------------|--------------------|----------------|--------------|
| 2,250°, 4 hrs. air-cooled  |            |                |                    |                |              |
| 2,000°, 4 hrs. air-cooled  |            |                |                    |                |              |
| 1,500°, 24 hrs. air-cooled |            |                |                    |                |              |
| 1,400°, 16 hrs. air-cooled | 1,700      | 38,000         | 20.5               | 3.8            | 2.3          |
| Same                       | 1,700      | 33,000         | 47.8               | 6.0            | 5.0          |
| 2,250°, 4 hrs. air-cooled  |            |                |                    |                |              |
| 1,550°, 24 hrs. air-cooled |            |                |                    |                |              |
| 2,000°, 4 hrs. air-cooled  |            |                |                    |                |              |
| 1,400°, 16 hrs. air-cooled | 1,700      | 38,000         | 14.8               | 3.1            | 3.2          |
| Same                       | 1,700      | 33,000         | 48.1               | 3.9            | 3.3          |

|                 | Percent by wt. |
|-----------------|----------------|
| Carbon          | 0.086-0.095    |
| Chromium        | 7.96-8.09      |
| Molybdenum      | 5.95-6.07      |
| Tantalum        | 5.99-4.46      |
| Cobalt          | 9.88-10.92     |
| Titanium        | 0.84-1.06      |
| Aluminum        | 5.99-6.17      |
| Boron           | 0.012-0.015    |
| Zirconium       | 0.081-0.089    |
| Silicon         | <0.25          |
| Iron            | <0.035         |
| Nickel, balance |                |

These specimens were heat treated as follows: 4 hours at 2250° F., then air cooled, 4 hours at 2000° F., then air cooled, 24 hours at 1550° F., then air cooled and 16 hours at 1400° F. followed by air cooling.

Rupture tests were performed and gave the following results:

1800° F. 20,000 p.s.i. (93 hours with 7% elongation);  
1800° F. 24,000 p.s.i. (42 hours);  
1750° F. 30,000 p.s.i. (80 hours);  
1750° F. 28,000 p.s.i.;  
1600° F. 46,000 p.s.i. (119.7 hours—2.8% elongation and 2.5% reduction in area);  
1600° F. 36,000 p.s.i. (260 hours).

Tensile strength tests at 1400° F. gave the following results:

129,000 p.s.i. for 0.2% elongation;  
147,000 p.s.i. (ultimate strength with 4.7% elongation and 6.2% reduction in area).

At room temperature:

142,000 p.s.i. for 0.2% elongation;

Other tests indicate that the alloy specimens are better on rupture life by 35° to 50° than similar heat treated specimens of U-700, analysis given below.

One of these alloys was used to form first stage cast turbine blades which were uncoated and mounted in a gas turbine alternated with blades formed from a standard alloy, U-700 coated with "Jo-Coat" a standard blade coating.

The alloy compositions were:

| 50         | Example 6A, percent | U-700 (Specification), percent |
|------------|---------------------|--------------------------------|
| Carbon     | 0.095               | 0.03-0.10                      |
| Manganese  | 0.03                | <0.15                          |
| Zirconium  | 0.052               | ≤0.015                         |
| Sulfur     | 0.002               | ≤0.20                          |
| Cobalt     | 10.92               | 17-20                          |
| Chromium   | 7.96                | 14-16                          |
| Titanium   | 0.84                | 2.75-3.75                      |
| Molybdenum | 6.00                | 4.5-5.5                        |
| Aluminum   | 6.15                | 3.75-4.25                      |
| Boron      | 0.012               | 0.025-0.035                    |
| Tantalum   | 4.46                |                                |
| Nickel     | Balance             | Balance                        |

In a standard, low-cycle, thermal fatigue test in the first stage of a gas turbine of the airplane type, the blades were operated at a temperature somewhat in excess of 1800° F., for 1000 cycles, each cycle consisting of 2 minutes of hot operation followed by 8 minutes of cold operation.

At the conclusion of the 1000 cycle test, alloys substantially in accordance with the analysis of Example 6A, showed the following properties:

Average blade extension 50% of the extension of similar blades of Alloy U-700.

Maximum blade extension was 40% of the maximum blade extension of blades of Alloy U-700.

75

Stator vanes working with the rotor blades were provided formed from the alloy of Example 6A, alloy WI-52 and SM 302. At 1820° F. with the vanes in alternating sequence, all blades being tested showed bowing after 1000 cycles of test operation.

SM 302 10 times that of vanes of the alloy of Example 6A  
WI-52 5 times that of vanes of the alloy of Example 6A

In another low cycle thermal fatigue test with a turbine inlet temperature of 1810° F. after 1440 cycles, the bowing of vanes of the alloy of Example 6A was only one-fourth that of alloy WI-52.

5

At 1400° F., tensile strength specimens showed an ultimate strength of 131,000 p.s.i. with 4.0% elongation and 4.7% reduction in area and a yield strength with 0.2% elongation of 115,000 p.s.i.

At 1400° F. tensile strength specimens of the cast alloy maintained under continuously applied axial stress of 85,000 p.s.i. ruptured after 39.3 hours, and exhibited an

10

At 1400° F. tensile strength specimens of the cast alloy maintained under continuously applied axial stress of 85,000 p.s.i. ruptured after 39.3 hours, and exhibited an

## WEIGHT PERCENT OF ALLOY CONSTITUENTS

|            | Example |         |         |         |         |
|------------|---------|---------|---------|---------|---------|
|            | No. 11  | No. 12  | No. 13  | No. 14  | No. 15  |
| Carbon     | 0.1     | 0.1     | 0.2     | 0.1     | 0.13    |
| Chromium   | 8.2     | 8.2     | 8.2     | 8.2     | 8.2     |
| Molybdenum | 6.0     | 6.0     | 6.0     | 6.0     | 6.0     |
| Tantalum   | 4.2     | 4.2     | 4.2     | 4.2     | 4.0     |
| Mo + Ta    | 10.2    | 10.2    | 10.2    | 10.2    | 10.0    |
| Cobalt     | 10.0    | 10.0    | 10.0    | 10.0    | 9.9     |
| Titanium   | 1.5     | 1.0     | 1.0     | 1.0     | 1.0     |
| Aluminum   | 6.0     | 7.0     | 6.0     | 6.0     | 6.1     |
| Ti + Al    | 7.5     | 8.0     | 7.0     | 7.0     | 7.1     |
| Boron      | 0.012   | 0.012   | 0.012   | 0.046   | 0.012   |
| Zirconium  | 0.08    | 0.08    | 0.08    | 0.08    | 0.1     |
| Iron       |         |         |         |         | 2.1     |
| Vanadium   |         |         |         |         |         |
| Tungsten   | Balance | Balance | Balance | Balance | Balance |
| Nickel     |         |         |         |         |         |

The alloy of Example No. 11 had the following mechanical properties:

Standard tensile strength test specimens at room temperature showed a tensile strength of 157,000 p.s.i., with 10.0% elongation, and a yield strength with 0.2% elongation of 126,000 p.s.i.

At 1400° F. tensile strength test specimens showed an ultimate strength of 126,000 p.s.i. an elongation of 5.0% and 7.8% reduction in area; and a yield strength at 0.2% elongation of 122,000 p.s.i.

At 1400° F. tensile strength specimens of the cast alloy maintained under continuously applied axial stress of 85,000 p.s.i. ruptured after 201.2 hours, and exhibited an elongation after rupture of 5.1%, and a reduction in area of 5.9%.

At 1800° F., and at a loading of 29,000 p.s.i., specimens ruptured after 37.5 hours, showing 5.2% elongation, and an area reduction of 3.8%.

At 1900° F. and a loading of 18,000 p.s.i., specimens ruptured after 38.5 hours with an elongation of 3.1% and an area reduction of 2.9%.

The alloy of Example No. 12 had the following mechanical properties:

Standard tensile strength test specimens at room temperature showed a tensile strength of 139,000 p.s.i., with 5.0% elongation, and an area reduction of 8.2%; and a yield strength with 0.2% elongation of 122,000 p.s.i.

At 1400° F., tensile strength specimens showed an ultimate strength of 144,000 p.s.i., an elongation of 5.0% and a reduction in area of 7.8%; and a yield strength with 0.2% elongation of 122,000 p.s.i.

At 1400° F. tensile strength specimens of the cast alloy maintained under continuously applied axial stress of 85,000 p.s.i. ruptured after 105.0 hours, and exhibited an elongation after rupture of 5.3% and an area reduction of 5.1%.

At 1800° F., and at a loading of 29,000 p.s.i., specimens ruptured after 32.4 hours, showing 4.0% elongation and an area reduction of 3.4%.

At 1900° F. and 18,000 p.s.i. rupture occurred after 29.0 hours with 3.8% elongation and 3.5% reduction in area.

The alloy of Example No. 13 had the following mechanical properties:

Standard tensile strength test specimens at room temperature showed a tensile strength of 138,000 p.s.i., with 7.0% elongation and an area reduction of 7.8%; and a yield strength with 0.2% elongation of 118,000 p.s.i.

At 1400° F., tensile strength specimens showed an ultimate strength of 131,000 p.s.i. with 4.0% elongation and 4.7% reduction in area and a yield strength with 0.2% elongation of 115,000 p.s.i.

At 1400° F. tensile strength specimens of the cast alloy maintained under continuously applied axial stress of 85,000 p.s.i. ruptured after 39.3 hours, and exhibited an

elongation after rupture of 2.0%, and a reduction in area of 1.9%.

At 1800° F., and at a loading of 29,000 p.s.i., specimens ruptured after 35.5 hours, showing 6.7% elongation, and an area reduction of 7.4%.

At 1900° F. and at a loading of 18,000 p.s.i. specimens ruptured after 37.7 hours and showed 8.3% elongation and a reduction in area of 8.1%.

The alloy of Example No. 14 had the following mechanical properties:

Standard tensile strength test specimens at room temperature showed a tensile strength of 136,000 p.s.i., with 7.0% elongation, an area reduction of 6.5%; and a yield strength with 0.2% elongation of 113,000 p.s.i.

At 1400° F. tensile strength specimens showed an ultimate rupture strength of 129,000 p.s.i. with 7% elongation and 6.5% reduction in area; and with 0.2% yield strength at 114,000 p.s.i.

At 1400° F. tensile strength specimens of the cast alloy maintained under continuously applied axial stress of 85,000 p.s.i. ruptured after 139.6 hours, and exhibited an elongation after rupture of 2.3% with 3.5% reduction in area.

At 1800° F. and at a loading of 29,000 p.s.i., specimens ruptured after 38.5 hours, showing 9.6% elongation, and a reduction in area of 10.0%.

At 1900° F. at a loading of 18,000 p.s.i., specimens ruptured after 34.1 hours, with an elongation of 7.6% and a reduction in area of 9.1%.

The alloy of Example No. 15 had the following mechanical properties:

Standard tensile strength test specimens at room temperature showed a tensile strength of 148,000 p.s.i., with 6.0% elongation and 10.2% reduction in area; and a yield strength with 0.2% elongation of 122,000 p.s.i.

At 1400° F. tensile strength specimens showed an ultimate rupture strength of 133,000 p.s.i. with 2.0% elongation and 3.0% area reduction; and 0.2% yield strength of 125,000 p.s.i.

At 1400° F. tensile strength specimens of the cast alloy maintained under continuously applied axial stress of 85,000 p.s.i. ruptured after 113.1 hours, and exhibited an

elongation after rupture of 5.9% and an area reduction of 4.7%.

At 1800° F. and at a loading of 29,000 p.s.i. specimens ruptured after 8.4 hours, showing 6.3% elongation, and an area reduction of 5.8%.

At 1900° F. and at a loading of 18,000 p.s.i. specimens ruptured after 13.4 hours with 3.8% elongation and 2.7% reduction in area.

While the alloy of Example No. 15 does not exhibit unusually good tensile and rupture properties at high temperature, it is an excellent alloy which can be rolled, forged or extruded to form shielding and to provide sheeting which have good corrosion and erosion properties at high temperatures.

p.s.i., with 5.0% elongation and 8.0% reduction in area at rupture and a yield strength with 0.2% elongation of 125,000 p.s.i.

At 1400° F. tensile strength specimens of the cast alloy maintained under continuously applied axial stress of 85,000 p.s.i. ruptured after 117.0 hours, and exhibited an elongation after rupture of 4.4%, and an area reduction of 5.1%. At 1600° F. and a loading of 55,000 p.s.i., the specimen ruptured after 78.0 hours, showing an elongation of 5.5% after rupture and an area reduction of 5.4%.

At 1700° F. and a loading of 40,000 p.s.i., the specimen ruptured after 67.4 hours with 6.8% elongation and 5.6% reduction in area.

When tested at 2000° F. and a loading of 10,000 p.s.i.,

#### WEIGHT PERCENT OF ALLOY CONSTITUENTS

|            | Example |         |         |         |         |
|------------|---------|---------|---------|---------|---------|
|            | No. 16  | No. 17  | No. 18  | No. 19  | No. 20  |
| Carbon     | .1      | 0.1     | 0.1     | 0.1     | 0.1     |
| Chromium   | 8.0     | 8.3     | 4.5     | 5.2     | 5.5     |
| Molybdenum | 4.7     | 6.1     | 4.0     | 3.0     | 6.0     |
| Tantalum   | 7.3     | 3.7     | 8.2     | 4.1     | 4.0     |
| Mo + Ta    | 8.0     | 9.8     | 12.2    | 7.1     | 10.0    |
| Cobalt     | 10.3    | 13.50   | 12.0    | 15.4    | 13.3    |
| Titanium   | 1.1     | 1.1     | 1.1     | 1.5     | 1.15    |
| Aluminum   | 6.0     | 5.95    | 6.0     | 7.3     | 5.3     |
| Ti + Al    | 7.1     | 7.05    | 7.1     | 8.8     | 6.45    |
| Boron      | 0.013   | 0.011   | 0.01    | 0.02    | 0.01    |
| Zirconium  | 0.10    | 0.1     | 0.11    | 0.09    | 0.09    |
| Nickel     | Balance | Balance | Balance | Balance | Balance |

The alloy of Example No. 16 had the following mechanical properties:

Standard tensile strength test specimens at room temperature showed a tensile strength of 137,500 p.s.i., with 7.0% elongation and 10.0% reduction in area, and a yield strength with 0.2% elongation of 116,250 p.s.i.

At 1400° F. tensile strength specimens showed an ultimate strength of 143,000 p.s.i. with 116,250 p.s.i. elongation 6.0% and reduction in area of 11.0%.

At 1400° F. tensile strength specimens of the cast alloy maintained under continuously applied axial stress of 94,000 p.s.i. ruptured after 108.7 hours, and exhibited an elongation after rupture of 3.0%, and prior elongation of 2.005%. At 1800° F. and a loading of 29,000 p.s.i., specimens ruptured after 75.1 hours, showing an elongation of 8.0% after rupture. When tested at 1900° F. and a loading of 18,000 p.s.i., the specimens ruptured after 107.3 hours, with 7.5% elongation after rupture.

At 1400° F. and 85,000 p.s.i. the specimens ruptured at 340.5 hours with an elongation of 3.5% and prior extension of 2.42%.

Long time creep and rupture tests run on virgin-melt specimens of alloy of Example 16 gave the following data:

a specimen ruptured after 61.8 hours, with 20.7% elongation after rupture and 17.8% area reduction.

Another specimen of substantially the same composition as the alloy of Example No. 17 exhibited the following properties:

Standard tensile strength test specimens at 1400° F. temperature showed a tensile strength of 141,000 p.s.i., with 5.0% elongation, 8.0% reduction in area and a yield strength with 0.2% elongation of 119,000 p.s.i.

At 1400° F. tensile strength specimens of the cast alloy maintained under continuously applied axial stress of 85,000 p.s.i. ruptured after 171.5 hours, and exhibited an elongation after rupture of 3.0%, and an area reduction of 3.1%. At 1800° F. and a loading of 29,000 p.s.i., specimens ruptured after 52.7 hours, showing an elongation of 5.0% after rupture and an area reduction of 3.9%. When tested at 1900° F. and a loading of 18,000 p.s.i., the specimens ruptured after 61.0 hours, with 6.0% elongation after rupture and 6.3% reduction.

After being subjected to a creep test at 1400° F., with an axial stress of 85,000 p.s.i. for 326.4 hours, the specimen showed an elongation of 5.4% and a reduction in area of 4.7% and failed at 328.0 hours.

| Temp., ° F.                      | 1,600    | 1,650   | 1,700  | 1,750  | 1,800  | 1,850  |
|----------------------------------|----------|---------|--------|--------|--------|--------|
| P.s.i.                           | 29,000   | 29,000  | 29,000 | 29,000 | 29,000 | 29,000 |
| Prior Extension hrs.             | 2,373.6+ | 1,931.2 | 645.2  | 141.1  | 75.0   | 13.9   |
| Prior Extension (creep), percent | 0.992    | 8.846   | 6.198  | 4.319  | 2.977  |        |
| Final hrs.                       | 1,931.4  | 647.0   | 143.5  | 75.0   | 15.0   |        |
| Final Elong., percent            | 10.5     | 8.0     | 6.6    | 8.0    | 8.4    |        |
| Final R.A., percent              | 13.3     | 8.6     | 8.5    | 8.5    | 7.8    |        |

The alloy of Example No. 17 had the following mechanical properties:

Standard tensile strength test specimens at room temperature showed an ultimate tensile strength of 140,000 p.s.i.

An alloy similar to the alloy of Example 17, after heat treatment for 4 hours at 2250° F., followed by air cooling 4 hours at 2000° F., followed by air cooling, followed by 24 hours at 1550° F. and air cooling, and finally by

heating at 1400° F. for 16 hours followed by air cooling, was the source of hot-forged specimens which gave the following data:

## RUPTURE TESTS

| Temp., ° F. | Load, p.s.i. | Hours | El., percent     |
|-------------|--------------|-------|------------------|
| 1,750       | 28,000       | 60.0  | 4.3              |
| 1,750       | 26,000       | 98.0  | 7.8              |
| 1,800       | 24,000       | 42.0  |                  |
| 1,800       | 20,000       | 93.0  | 7.2              |
| 1,800       | 18,000       | 154.0 | 7.2              |
| 1,850       | 18,000       | 53.0  | 7.4              |
| 1,850       | 16,000       | 97.0  | 9.2              |
| 1,600       | 54,000       | 14.7  | 2.3              |
| 1,600       | 50,000       | 42.5  | 1.7              |
| 1,600       | 46,000       | 119.7 | 2.8              |
| 1,600       | 36,000       | 260.0 | ( <sup>1</sup> ) |
| 1,675       | 44,000       | 18.0  |                  |

<sup>1</sup> Test stopped.

perature showed a tensile strength of 145,000 p.s.i., with 14.0% elongation and 13.7% reduction in area; and a yield strength with 0.2% elongation of 110,000 p.s.i.

At 1400° F., the specimen showed an ultimate tensile strength of 113,000 p.s.i. and on rupture an elongation of 3.0%, an area reduction of 9.1%; and a yield strength at .2% elongation of 105,000 p.s.i.

At 1800° F. tensile strength specimens of the cast alloy maintained under continuously applied axial stress of 29,000 p.s.i. ruptured after 43.8 hours, and exhibited an elongation after rupture of 6.0%, and an area reduction of 11.0%.

At 1900° F. and a loading of 18,000 p.s.i., specimens ruptured after 68.3 hours, showing an elongation of 8.0% after rupture and an area reduction of 13.0%.

Alloys corresponding to Example No. 20 with its high cobalt content respond to extrusion and have been extruded at a 16:1 ratio, from a 5" ingot to a 1/2" bar.

## WEIGHT PERCENT OF ALLOY CONSTITUENTS

| Example              | No. 21  | No. 22  | No. 23  | No. 24  | No. 25  | No. 26  | No. 27  |
|----------------------|---------|---------|---------|---------|---------|---------|---------|
| Carbon               | 0.1     | 0.08    | 0.07    | 0.1     | 0.09    | 0.12    | 0.16    |
| Chromium             | 8.2     | 8.0     | 7.8     | 7.7     | 9.7     | 8.00    | 12.00   |
| Molybdenum           | 6.0     | 8.0     | 5.8     | 4.0     | 3.0     | 4.00    | 3.27    |
| Tantalum             | 4.0     | 4.1     | 6.2     | 7.7     | 7.2     | 8.00    | 7.50    |
| Mo plus Ta           | 10.0    | 12.1    | 12.0    | 11.7    | 10.5    |         |         |
| Cobalt               | 10.0    | 10.1    | 9.9     | 10.1    | 10.2    | 14.00   | 10.15   |
| Titanium             | 1.0     | 0.9     | 0.8     | 1.2     | 1.1     | 1.0     | 1.04    |
| Aluminum             | 6.0     | 5.8     | 5.9     | 6.0     | 6.2     | 6.0     | 6.31    |
| Ti plus Al           | 7.0     | 6.7     | 6.7     | 7.2     | 7.3     |         |         |
| Boron                | 0.012   | 0.024   | 0.024   | 0.014   | 0.014   | 0.012   | 0.011   |
| Zirconium            | 0.08    | 0.06    | 0.07    | 0.1     | 0.1     | .09     | 0.09    |
| Nickel (essentially) | Balance | Balance | Balance | Balance | Balance | Balance | Balance |

The alloy of Example No. 18 had the following mechanical properties:

Standard tensile strength test specimens at room temperature showed a tensile strength of 141,000 p.s.i., with a 5.0% elongation and 7.8% reduction in area; and a yield strength with 0.2% elongation of 130,000 p.s.i.

At 1900° F. a tensile strength specimen of the cast alloy maintained under continuously applied axial stress of 29,000 p.s.i. ruptured after 38.9 hours, and exhibited an elongation after rupture of 7.0%, and an area reduction of 4.8%.

The alloy of Example No. 19 had the following mechanical properties:

Standard tensile strength test specimens at room temperature showed a tensile strength of 125,000 p.s.i., with 13.0% elongation and 21.0% reduction in area; and a yield strength with 0.2% elongation of 95,000 p.s.i.

At 1400° F., test specimens showed an ultimate tensile strength of 129,000 p.s.i. with an elongation of 5.0% and a reduction in area of 6.2%.

At 1800° F. tensile strength specimens of the cast alloy maintained under continuously applied axial stress of 29,000 p.s.i. ruptured after 37.4 hours, and exhibited an elongation after rupture of 10.5%, and an area reduction of 4.8%.

At 1900° F. and a loading of 18,000 p.s.i., specimens ruptured after 36.3 hours, showing an elongation of 7.0% after rupture and an area reduction of 6.0%.

The alloy of Example No. 20 had the following mechanical properties:

Standard tensile strength test specimens at room tem-

45 Tensile data of the alloy of Example No. 21 follows:

| Temp., ° F. | 0.2% Yield, p.s.i. | Ultimate Tensile Strength, p.s.i. | Elongation in percent | Reduction in area in percent |
|-------------|--------------------|-----------------------------------|-----------------------|------------------------------|
| 1,000       | 126,000            | 146,000                           | 7.0                   | 13.8                         |
| 1,100       | 128,000            | 150,000                           | 6.0                   | 8.7                          |
| 1,200       | 134,000            | 147,000                           | 6.0                   | 7.0                          |
| 1,300       | 120,000            | 147,000                           | 5.0                   | 5.0                          |
| 1,400       | 117,000            | 136,000                           | 5.0                   | 4.6                          |
| 1,500       | 122,000            | 129,000                           | 4.0                   | 3.0                          |
| 1,600       | 106,000            | 108,000                           | 4.0                   | 4.0                          |
| 1,700       | 70,000             | 105,000                           | 4.0                   | 3.0                          |
| 1,800       | 51,000             | 80,000                            | 6.0                   | 7.0                          |
| 1,900       | 46,000             | 58,000                            | 4.0                   | 5.0                          |
| 2,000       | 31,000             | 39,000                            | 8.0                   | 9.0                          |
| 2,100       | 14,000             | 18,000                            | 14.0                  | 14.0                         |
| 2,200       | 5,700              | 6,200                             | 40.0                  | 44.0                         |

Generally alloys that tend to show good strength at 1700° F. to 1800° F. fall off markedly when reaching 1900° F. with a load of 20,000 p.s.i. or more. The alloys of the present invention generally average 30 or more hours at 1900° F. with 20,000 p.s.i. and with an elongation of 5.0% or better. Further, alloys such as the alloy of Example No. 21 have more than a 200 hour life at 2000° F. 8,000 p.s.i., with 9.0% elongation and great strength between 1200° F. and 1700° F.

Test results on the alloy of Example No. 21 are shown in the following table:

| Temperature, ° F. | Rupture Load, p.s.i. | Hours    | Elongation in percent | Reduction in area, percent |
|-------------------|----------------------|----------|-----------------------|----------------------------|
| 1,200             | 105,000              | 1,280.0+ | 3.0                   | 6.2                        |
| 1,300             | 95,000               | 306.9    | 2.5                   | 4.8                        |
| 1,400             | 85,000               | 217.7    | 4.3                   | 3.9                        |
| 1,500             | 65,000               | 376.7    | 4.0                   | 4.0                        |
| 1,500             | 70,000               | 174.1    | 4.0                   | 3.9                        |
| 1,500             | 75,000               | 83.6     | 4.0                   | 4.8                        |
| 1,600             | 50,000               | 166.4    | (1)                   |                            |
| 1,600             | 55,000               | 180.6    | 4.5                   | 7.1                        |
| 1,600             | 60,000               | 67.6     | 4.9                   | 5.1                        |
| 1,700             | 33,000               | 168.8    | (1)                   |                            |
| 1,700             | 40,000               | 83.1     | 3.0                   | 4.8                        |
| 1,800             | 29,000               | 59.2     | 3.0                   | 3.1                        |
| 2,000             | 10,000               | 77.8     | 2.0                   |                            |
| 2,000             | 8,000                | 192.8    | 3.0                   |                            |
| 2,100             | 5,000                | 82.0     | 5.1                   |                            |
| 2,100             | 3,800                | 79.5     | 4.0                   |                            |

<sup>1</sup> Stopped test at 1% extension.

The alloy of Example No. 21 is among the preferred vacuum melted alloys of this invention and standard test specimens show excellent oxidation and erosion resistance when subjected to a jet engine burner-can flame at rates higher than 0.6 Mach, at a temperature of 2100° F. for 200 hours in an uncoated condition. The following table compares such data with similar tests on specimens made of "alloy #101."

Grams  
Weight loss after 200 hrs. of Example No. 21 ----- 0.3  
Weight loss after 200 hrs. of Alloy #101 ----- 1.0

Similar tests on specimens coated with "Jo-Coat" (a standard gas turbine blade coating) but at 2100° F. gave the following comparative data:

Grams  
Weight loss after 200 hrs. of Example No. 21 ----- 0.06  
Weight loss after 200 hrs. of Alloy #101 ----- 0.10

The following gives the results of tests of the static oxidation rate at 2200° F. for 100 hours for the alloy of Example No. 21 compared with alloys #100 and #101, on specimens machined to identical length and shape:

#### WEIGHT GAIN MG./CM.<sup>2</sup>

| Alloy               | 25 hrs. | 50 hrs. | 100 hrs. |
|---------------------|---------|---------|----------|
| Example No. 21, mg. | +7.0    | +10.4   | +20.7    |
| #100, mg.           | +255.0  | +313.0  | +591.0   |
| #101, mg.           | +28.4   | +50.0   | +117.0   |

The alloy of Example No. 21 of the present invention thus shows approximately one-sixth the oxidation at 2200° F. of alloy #101 and approximately one-thirtieth that of alloy #100.

Other tests on the alloy of Example No. 21 gave the following data:

[0.6 Mach jet engine burner can flame erosion test at 2100° F.]

| Sample Weight           | 100 hrs., g. loss | 200 hrs., g. loss |
|-------------------------|-------------------|-------------------|
| Example No. 21          | 0.15              | 0.30              |
| Alloy #101              | 0.40              | 0.95              |
| Example No. 21 (coated) | 0.04              |                   |
| Alloy #101 (coated)     | 0.11              |                   |

Micro examination of the test bars showed no grain boundary attack for the alloy of Example No. 21, while alloy #101 showed positive boundary attack. Also, the coating ("Jo-Coat") married better to the alloy of Example No. 21 than to the alloy #101.

A paddle test, to determine susceptibility to cracking upon alternate heating and water quenching was conducted with the test specimens being heated to various temperatures for 1 minute, then quenched with cold

water for 1/2 minute, with a water flow at 250 pounds per hour, the test specimens being rotated at 1750 r.p.m. gave the following comparative data, expressed in hours before incipient cracking was observed:

5

|                | 2,000° F., hrs. | 1,900° F., hrs. | 1,800° F., hrs. |
|----------------|-----------------|-----------------|-----------------|
| Example No. 21 | 150             | 350             | 900             |
| Example No. 12 | 200             | 400             | 1150            |
| Alloy #100     | 100             | 300             | 500             |
| Alloy #101     | 100-150         | 100-400         | 600-1,000       |
| Alloy #102     | 100-200         | 250-400         | 500-700         |

15

Comparative static oxidation tests of a test specimen of the present invention, compared with conventional alloys gave the following results at 2200° F.

| 20              | Static oxidation tests at 2,200° F. | Gms./cm. <sup>2</sup> | Total loss |
|-----------------|-------------------------------------|-----------------------|------------|
| Alloy #101:     |                                     |                       |            |
| Original weight |                                     | 3.4830                |            |
| After 24 hours  |                                     |                       | -.0310     |
| After 148 hours |                                     |                       | -.1064     |
| Alloy #102:     |                                     |                       |            |
| Original weight |                                     | 3.2516                |            |
| After 24 hours  |                                     |                       | -.0086     |
| After 148 hours |                                     |                       | -.0340     |
| Alloy #100:     |                                     |                       |            |
| Original weight |                                     | 3.1306                |            |
| After 24 hours  |                                     |                       | -.0144     |
| After 148 hours |                                     |                       | -.0502     |
| Example No. 21: |                                     |                       |            |
| Original weight |                                     | 3.3736                |            |
| After 24 hours  |                                     |                       | +.0010     |
| After 148 hours |                                     |                       | -.0472     |

35 The alloy of Example No. 22 had the following mechanical properties:

Standard tensile strength test specimens at room temperature showed a tensile strength of 133,000 p.s.i., with 4.0% elongation and 7.6% reduction in area; and a yield strength with 0.2% elongation of 126,000 p.s.i.

40 At 1900° F. tensile strength specimens of the cast alloy maintained under continuously applied axial stress of 18,000 p.s.i. ruptured after 35.4 hours, and exhibited an elongation after rupture of 2.0%, and an area reduction of 2.0%.

45 The alloy of Example No. 23 had the following mechanical properties:

Standard tensile strength test specimens at room temperature showed an ultimate tensile strength of 144,000 p.s.i., with 4.0% elongation and 5.3% reduction in area, and a yield strength with 0.2% elongation of 131,000 p.s.i.

50 At 1900° F. tensile strength specimens of the cast alloy maintained under continuously applied axial stress of 18,000 p.s.i. ruptured after 30.4 hours, and exhibited an elongation after rupture of 4.0%, and an area reduction of 3.1%.

55 After being subjected to a static oxidation test at 2000° F., a weight loss was observed of 0.0182 gram on the standard test specimen.

60 A standard salt erosion test with jet fuel at 1900° F. and 1000' r.p.m. conducted for 50 hours gave the following results compared with similar tests on alloys #101 and #102:

#### 65 SALT TEST WITH JET FUEL—1900° F.—50 HOURS—1000 R.P.M. [1st 25 hours]

| 70          | Alloy of Example No. 23 |        | Alloy #101<br>Uncoated | Alloy #102<br>Uncoated |
|-------------|-------------------------|--------|------------------------|------------------------|
|             | Uncoated                | Coated |                        |                        |
| Start grams | 56.43                   | 53.90  | 58.34                  | 54.22                  |
| 25 hrs.     | 56.38                   | 53.90  | 57.47                  | 53.93                  |
| Weight loss | 0.05                    | 0.00   | 0.87                   | 0.29                   |

75

[2nd 25 hours]

|                                       |       |       |       |       |
|---------------------------------------|-------|-------|-------|-------|
| Start grams.....                      | 56.38 | 53.90 | 57.47 | 53.93 |
| 25 hrs.....                           | 55.38 | 53.90 | 55.87 | 52.89 |
| Weight loss.....                      | 1.00  | 0.00  | 1.60  | 1.04  |
| Total Weight loss at end of test..... | 1.05  | 0.00  | 2.47  | 1.33  |

The alloy of Example No. 24 had the following mechanical properties:

Standard tensile strength test specimens at room temperature showed an ultimate tensile strength of 129,500 p.s.i. with 6.0% elongation and 11.0% reduction in area; and a yield strength with 0.2% elongation of 114,000 p.s.i.

At 1400° F. the ultimate tensile strength was 140,000 p.s.i. with 4.4% elongation and 7.0% reduction in area. The 0.2% elongation at 1400° F. was reached at 113,000 p.s.i.

At 1400° F. tensile strength specimens of the cast alloy maintained under continuously applied axial stress of 85,000 p.s.i. ruptured after 215.6 hours, and exhibited an elongation after rupture of 2.2%, and an area reduction of 1.51%. At 1800° F. and a loading of 29,000 p.s.i., specimens ruptured after 58.6 hours, showing 6.5% elongation. When tested at 1900° F. and a loading of 18,000 p.s.i., the specimens ruptured after 78.0 hours, with 7.5% elongation after rupture.

A similar alloy to Example 24 from a different heat and

having a specific analysis as follows, gave the following data:

|            |       |
|------------|-------|
| Carbon     | 0.18  |
| Chromium   | 7.90  |
| Molybdenum | 4.03  |
| Tantalum   | 7.76  |
| Cobalt     | 9.90  |
| Boron      | 0.012 |
| Zirconium  | 0.10  |
| Titanium   | 1.13  |
| Aluminum   | 5.90  |
| Manganese  | <0.20 |

Balance, essentially nickel.

## ROOM TEMPERATURE TENSILE STRENGTH

| Ultimate, p.s.i. | 0.2% Elongation, p.s.i. | Elongation, percent | Red. in Area, percent |
|------------------|-------------------------|---------------------|-----------------------|
| 135,250          | 109,000                 | 9.5                 | 11.5                  |

## RUPTURE TESTS

|                         | Hrs. | Prior Hrs. | Percent Elong. | Red. in Area, percent |
|-------------------------|------|------------|----------------|-----------------------|
| 1,400° F./94,000 p.s.i. | 41.2 | 40.1       | 1.9            | 3.9                   |
| 1,800° F./29,000 p.s.i. | 45.8 | -----      | 7.6            | 10.1                  |
| 1,900° F./18,000 p.s.i. | 40.6 | -----      | 9.0            | -----                 |

Test results on the alloys of Examples Nos. 24 and 25 are shown in the following tables:

## ROOM TEMPERATURE TENSILE STRENGTH TESTS

| Example  | .2% Elong., p.s.i. | Ult., p.s.i. | Elongation, percent | Reduction in area (percent) |
|----------|--------------------|--------------|---------------------|-----------------------------|
| No. 24:  |                    |              |                     |                             |
| (1)----- | 120,500            | 147,000      | 6.5                 | 12.5                        |
| (2)----- | 120,000            | 149,250      | 8.5                 | 12.5                        |
| No. 25:  |                    |              |                     |                             |
| (1)----- | 118,250            | 142,250      | 8.0                 | 12.5                        |
| (2)----- | 117,500            | 147,000      | 9.0                 | 13.5                        |

## 1400° F. TENSILE STRENGTH TESTS

|             |         |         |     |     |
|-------------|---------|---------|-----|-----|
| No. 24----- | 117,250 | 143,500 | 5.0 | 8.0 |
| No. 25----- | 117,250 | 142,000 | 4.0 | 8.0 |

## RUPTURE TESTS

|             | Temp., ° F. | P.s.i. | Hours | Elongation, percent | Reduction in area, percent |
|-------------|-------------|--------|-------|---------------------|----------------------------|
| No. 24----- | 1,400       | 94,000 | 111.7 | 2.5                 | Prior 1.09.                |
| No. 25----- | 1,400       | 94,000 | 113.9 | 3.7                 | 2.5 Prior 1.77.            |
| No. 24----- | 1,400       | 85,000 | 391.3 | 3.7                 | 5.0 Prior 2.04.            |
| No. 25----- | 1,400       | 85,000 | 414.0 | 4.0                 | 8.0 Prior 2.26.            |
| No. 24----- | 1,800       | 29,000 | 74.6  | 8.0                 | 6.5                        |
| No. 25----- | 1,800       | 29,000 | 67.8  | 9.5                 | 9.5                        |
| No. 24----- | 1,900       | 18,000 | 89.2  | 8.0                 | 8.5                        |
| No. 25----- | 1,900       | 18,000 | 65.2  | 6.0                 | 8.0                        |

|             | Temp., ° F. | P.s.i. | Hours | Total Elongation, percent | Hours Prior to Rupture | Creep Extension Prior to Rupture |
|-------------|-------------|--------|-------|---------------------------|------------------------|----------------------------------|
| No. 24----- | 1,400       | 94,000 | 137.9 | 4.1                       | 136.7                  | 2.233                            |
| No. 25----- | 1,400       | 94,000 | 113.4 | 5.2                       | 112.5                  | 2.2728                           |
| No. 24----- | 2,000       | 10,000 | 89.9  | 8.2                       | 89.0                   | 3.401                            |
| No. 25----- | 2,000       | 10,000 | 139.8 | 9.0                       | 136.9                  | 1.728                            |
| No. 25----- | 2,100       | 7,000  | 14.0  | 15.0                      | -----                  | -----                            |
| No. 25----- | 2,150       | 7,000  | 6.9   | 3.8                       | -----                  | -----                            |
| No. 25----- | 2,200       | 4,000  | 23    | 6.4                       | -----                  | -----                            |

The alloy of Example No. 26 provides cast alloys which, in general, have unusually good oxidation and corrosion resistance, are superior in their resistance to sulfidation from fuel combustion, and have tensile and rupture properties which exceed existing specifications, and have the following mechanical properties:

Room temperature ultimate tensile strength 141,000 p.s.i., yield strength 108,500 p.s.i. with 7.5% elongation and reduction in area of 12.5%.

At 1400° F. tensile strength was 135,000 p.s.i. ultimate, 10 107,000 yield strength with 4.0% elongation and 8.5% reduction in area.

| Temp., °F. | P.s.i. | Hours | Percent Elong. | Prior Percent |
|------------|--------|-------|----------------|---------------|
| 1,400      | 85,000 | 178.9 | 5.0            | 2.94          |
| 1,400      | 94,000 | 31.6  | 3.5            | 1.03          |
| 1,800      | 29,000 | 22.3  | 7.0            | -----         |
| 1,900      | 18,000 | 36.5  | 7.0            | -----         |

The alloy of Example No. 27 provides cast alloys which, in general, have unusually good oxidation and corrosion resistance, are superior in their resistance to sulfidation from fuel combustion, and have tensile and rupture properties which exceed existing specifications, and have the following mechanical properties:

Room temperature ultimate tensile strength 136,250 p.s.i., yield strength 117,500 p.s.i. with 5.5% elongation and reduction in area of 9.5%.

At 1400° F. tensile strength was 141,000 p.s.i. ultimate, 30 114,000 yield strength with 4.5% elongation and 9.5% reduction in area.

| Temp., °F. | P.s.i. | Hours | Percent Elong. | Prior Percent |
|------------|--------|-------|----------------|---------------|
| 1,400      | 85,000 | 162.9 | 4.2            | 2.81          |
| 1,400      | 94,000 | 58.6  | 4.1            | 2.3           |
| 1,800      | 29,000 | 35.2  | 12.0           | -----         |
| 1,900      | 18,000 | 44.0  | 9.0            | -----         |

When heat treated for 10 to 80 hours in the temperature range of 1500° to 1700° F. this alloy No. 27 shows improved elongation properties and increased tensile strengths both at room temperatures and in the higher temperature ranges.

Further examples of alloys according to the present invention, in which there is a considerable variation in the relative amounts of titanium and aluminum, are as follows:

| Example    | Weight percent |       |       |       |       |
|------------|----------------|-------|-------|-------|-------|
|            | 28             | 29    | 30    | 31    | 32    |
| Carbon     | 0.12           | 0.1   | 0.1   | 0.06  | 0.05  |
| Chromium   | 8.0            | 7.9   | 8.0   | 7.85  | 8.05  |
| Molybdenum | 5.1            | 5.0   | 5.1   | 4.95  | 4.9   |
| Tantalum   | 7.1            | 6.9   | 7.1   | 6.90  | 6.9   |
| Cobalt     | 9.9            | 9.9   | 9.9   | 10.70 | 10.5  |
| Boron      | 0.014          | 0.013 | 0.014 | 0.017 | 0.017 |
| Zirconium  | 0.12           | 0.12  | 0.13  | 0.066 | 0.035 |
| Titanium   | 1.6            | 2.0   | 3.0   | 4.85  | 7.17  |
| Aluminum   | 6.0            | 5.1   | 3.9   | 1.99  | 0.0   |
| Iron       | <0.2           | <0.2  | <0.2  | <0.2  | <0.2  |
| Manganese  | <0.2           | <0.2  | <0.2  | <0.2  | <0.2  |

Balance all substantially nickel.

Test specimens of these alloys gave the following data on physical properties:

#### EXAMPLE 28.—TENSILE STRENGTH

|            | 2% Elong., p.s.i. | Ultimate, p.s.i. | Elong., percent | R.A., percent |
|------------|-------------------|------------------|-----------------|---------------|
| Room Temp. | 118,250           | 143,750          | 9.0             | 10.0          |
| 1,400°     | 118,250           | 141,750          | 7.5             | 11.5          |

#### RUPTURE

| Temp., °F. | P.s.i. | Hours | Elong., percent | R.A., percent |
|------------|--------|-------|-----------------|---------------|
| 1,400      | 94,000 | 96.5  | 3.7             | 4.8           |
| 1,400      | 94,000 | 83.6  | 3.9             | -----         |
| 1,400      | 85,000 | 334.2 | 4.5             | -----         |
| 1,800      | 29,000 | 54.1  | 4.2             | 6.9           |
| 1,800      | 29,000 | 60.0  | 6.0             | -----         |
| 1,900      | 18,000 | 86.5  | 6.5             | -----         |

#### EXAMPLE 29.—TENSILE STRENGTH

|            | 2% Elong., p.s.i. | Ultimate, p.s.i. | Elong., percent | R.A., percent |
|------------|-------------------|------------------|-----------------|---------------|
| Room Temp. | 121,000           | 148,250          | 9.0             | 13.5          |
| 1,400°     | 113,250           | 142,500          | 5.0             | 7.0           |

#### RUPTURE

| Temp., °F. | P.s.i. | Hours | Elong., percent | R.A., percent |
|------------|--------|-------|-----------------|---------------|
| 1,400      | 94,000 | 58.5  | 3.7             | 5.5           |
| 1,400      | 94,000 | 64.7  | 3.3             | -----         |
| 1,400      | 85,000 | 186.0 | 3.1             | -----         |
| 1,800      | 29,000 | 53.7  | 6.0             | 6.9           |
| 1,800      | 29,000 | 65.8  | 8.5             | -----         |
| 1,900      | 18,000 | 87.1  | 12.0            | -----         |

#### EXAMPLE 30.—TENSILE STRENGTH

|            | 2% Elong., p.s.i. | Ultimate, p.s.i. | Elong., percent | R.A., percent |
|------------|-------------------|------------------|-----------------|---------------|
| Room Temp. | 119,000           | 151,250          | 8.5             | 10.0          |
| 1,400° F.  | 106,000           | 140,000          | 4.0             | 7.0           |

| Temp., °F. | P.s.i. | Hours | Elong., percent | R.A., percent |
|------------|--------|-------|-----------------|---------------|
| 1,400      | 94,000 | 58.2  | 4.8             | 7.9           |
| 1,400      | 94,000 | 33.4  | 3.0             | -----         |
| 1,400      | 85,000 | 180.2 | 4.3             | -----         |
| 1,800      | 29,000 | 29.0  | 8.9             | 13.1          |
| 1,800      | 29,000 | 25.6  | 10.0            | -----         |
| 1,900      | 18,000 | 46.8  | 14.5            | -----         |

#### EXAMPLE 31.—TENSILE STRENGTH

|            | 2% Elong., p.s.i. | Ultimate, p.s.i. | Elong., percent | R.A., percent |
|------------|-------------------|------------------|-----------------|---------------|
| Room Temp. | 89,200            | 117,800          | 2.5             | 6.6           |
| 1,400° F.  | 90,100            | 137,500          | 3.6             | 5.6           |

#### EXAMPLE 32

|            | 2% Elong., p.s.i. | Ultimate, p.s.i. | Elong., percent | R.A., percent |
|------------|-------------------|------------------|-----------------|---------------|
| Room Temp. | 101,400           | 137,100          | 2.0             | 4.2           |
| 1,400° F.  | 86,500            | 115,000          | 2.0             | 3.7           |

Alloys such as those of Examples 28 to 31 show great ductility and are readily forged and exhibit excellent physical properties in the forged condition.

Still another example of an alloy according to the present invention has a low carbon content, about 6.0% molybdenum and a relatively high tantalum content, about 8.0%. A specific example (Example 33) of such an alloy is as follows:

|            | Percent by wt. |
|------------|----------------|
| Carbon     | 0.04           |
| Chromium   | 7.95           |
| Molybdenum | 5.85           |
| Tantalum   | 8.1            |

|                                    | Percent by wt. |
|------------------------------------|----------------|
| Cobalt                             | 11.0           |
| Boron                              | 0.01           |
| Zirconium                          | 0.048          |
| Titanium                           | 0.0            |
| Aluminum                           | 6.6            |
| Iron                               | <0.2           |
| Manganese                          | <0.2           |
| Balance, substantially all nickel. |                |

Specimens of this alloy showed the following physical properties:

TENSILE STRENGTH

|            | 2% Elong., p.s.i. | Ultimate, p.s.i. | Elong., percent | R.A., percent |
|------------|-------------------|------------------|-----------------|---------------|
| Room Temp. | 116,700           | 136,900          | 5.1             | 8.8           |
| 1,400° F.  | 117,300           | 158,700          | 5.1             | 8.1           |

RUPTURE

| Temp., ° F. | P.s.i. | Hours | Elong., percent | R.A., percent |
|-------------|--------|-------|-----------------|---------------|
| 1,400       | 94,000 | 57.3  | 6.3             | 9.4           |
| 1,800       | 29,000 | 37.9  | 5.2             | 6.4           |

Many of the alloys of the present invention are susceptible to heat treatment, and may be extruded and hot forged.

Illustrative of the properties of heat treated hot forged alloys corresponding to Example 3 are as follows:

(A) Heat treated for:

1 hour at 2290° F., then air cooled,  
100 hours at 1550° F., then air cooled,  
8 hours at 1900° F., then air cooled,  
24 hours at 1550° F., then air cooled,  
16 hours at 1400° F., then air cooled,  
and hot forged, ruptured at 1400° F. under 85,000 p.s.i. stress at 181.1 hours with 3.0% elongation and 5.7% reduction in area.

(B) Heat treated at 2290° F. for 1 hour, air cooled, 2000° F., 8 hours, air cooled, 24 hours at 1550° F., air cooled and 16 hours at 1400° F. followed by air cooling and hot forging ruptured at 193.3 hours with 85,000 p.s.i. stress at 1400° F. with 3.0% elongation and 2.7% reduction in area.

(C) Heat treated at 2250° F. for 1 hour, air cooled, 8 hours at 2000° F., air cooled, 16 hours at 1400° F. air cooled and 24 hours at 1650° F. followed by air cooling and hot forging, ruptured after 187.3 hours under 85,000 p.s.i. at 1400° F.

Forged, heat treated specimens of an alloy corresponding to Example 21 showed the following results on rupture tests:

HEAT TREATMENT

|   | ° F.  | P.s.i. | Hours | Percent El. | Percent R.A. |
|---|-------|--------|-------|-------------|--------------|
| A | 1,400 | 85,000 | 77.4  | 1.5         | 2.0          |
| B | 1,400 | 85,000 | 118.9 | 3.1         | 4.0          |
| C | 1,400 | 85,000 | 111.8 | 3.0         | 3.8          |

Specimens of a forged heat treated alloy corresponding to Example 25, showed the following results on rupture tests:

HEAT TREATMENT

|   | ° F.  | P.s.i. | Hours | Percent El. | Percent R.A. |
|---|-------|--------|-------|-------------|--------------|
| A | 1,400 | 85,000 | 196.1 | 3.1         | 6.6          |
| B | 1,400 | 85,000 | 192.9 | 3.1         | 8.0          |
| C | 1,400 | 85,000 | 109.1 |             |              |

In general, the alloys of the present invention may be extruded from a 5" or 6" ingot to as small as 1.1" and 6" ingots have been extruded and then rolled to form a  $\frac{5}{8}$ " bar as long as 40 feet.

In general, the alloys of the present invention are exceptionally well suited for use in the manufacture of blades for gas turbines and in such use are comparable in strength at 1800° to 1900° F. with blades made from alloy #101, are better than blades made from alloy #100 and much better than blades made from alloy #102.

The alloys of the present invention in general exhibit better static oxidation resistance than alloys #100, #101 and #102, and show no grain boundary attack at temperatures in excess of 2000° F. The present alloys produce excellent cast structures of great uniformity, which can be fully solutioned at about 2250° F. and can therefore be stabilized and aged for greater strength and ductility and are comparable with certain alloys containing 18% or more of cobalt, while having better overall properties including excellent oxidation and erosion properties.

The invention in its broader aspects is not limited to the specific steps, process and compositions shown and described but departures may be made therefrom within the scope of the accompanying claims without departing from the principles of the invention and without sacrificing its chief advantages.

What is claimed is:

30 1. A corrosion resistant nickel-base alloy for use at relatively high temperatures consisting essentially of the following elements in the weight percent ranges set forth:

|            | Percent |
|------------|---------|
| Chromium   | 5-12    |
| Molybdenum | 3-8     |
| Tantalum   | 2.3-10  |
| Cobalt     | 5-15.5  |
| Titanium   | 0-7     |
| Aluminum   | 0-8     |
| Carbon     | 0-0.25  |
| Boron      | 0-0.05  |
| Zirconium  | 0-1.0   |

the balance of the alloy being essentially nickel, the total of the molybdenum and tantalum being from 5% to 14% and the total of the aluminum and titanium being from 5% to 8.8%.

45 2. A corrosion resistant nickel-base alloy for use at relatively high temperatures consisting essentially of the following elements in the weight percent ranges set forth:

|            | Percent |
|------------|---------|
| Chromium   | 5-12    |
| Molybdenum | 3-8     |
| Tantalum   | 2.3-10  |
| Cobalt     | 5-15.5  |
| Titanium   | 0-2.5   |
| Aluminum   | 4-8     |
| Carbon     | 0-0.25  |
| Boron      | 0-0.05  |
| Zirconium  | 0-1.0   |

50 the balance of the alloy being essentially nickel, the total of the molybdenum and tantalum being from 5% to 14% and the total of the aluminum and titanium being from 5% to 8.8%.

65 3. A corrosion resistant nickel-base alloy for use at relatively high temperatures consisting essentially of the following elements in the weight percent ranges set forth:

|            | Percent |
|------------|---------|
| Chromium   | 7.5-12  |
| Molybdenum | 3-8     |
| Tantalum   | 2.3-10  |
| Cobalt     | 5-10.5  |
| Titanium   | 0-2.5   |
| Aluminum   | 5-7     |

|           | Percent |
|-----------|---------|
| Carbon    | 0-0.25  |
| Boron     | 0-0.05  |
| Zirconium | 0-1.0   |

the balance of the alloy being essentially nickel, the total of the molybdenum and tantalum being from 7% to 13% and the total of the aluminum and titanium being from 5.5% to 8%.

4. A corrosion resistant nickel-base alloy for use at relatively high temperatures consisting essentially of the following elements in the weight percent ranges set forth:

|            | Percent |
|------------|---------|
| Chromium   | 5-8     |
| Molybdenum | 3-6     |
| Tantalum   | 4-8     |
| Cobalt     | 10-15.5 |
| Titanium   | 1.0-2.3 |
| Aluminum   | 4.4-8   |
| Carbon     | 0-0.25  |
| Boron      | 0-0.05  |
| Zirconium  | 0-1.0   |

the balance of the alloy being essentially nickel, the total of the molybdenum and tantalum being from 7% to 12.2% and the total of the aluminum and titanium being from 5.4% to 8.8%.

5. A corrosion resistant nickel-base alloy for use at relatively high temperatures consisting essentially of the following elements in the weight percent ranges set forth:

|            | Percent   |
|------------|-----------|
| Chromium   | 7.5-8.5   |
| Molybdenum | 5.75-6.25 |
| Tantalum   | 4.0-4.5   |
| Cobalt     | 9.5-10.5  |
| Titanium   | 0.8-1.2   |
| Aluminum   | 5.75-6.25 |
| Carbon     | 0.08-0.13 |
| Boron      | 0.01-0.02 |
| Zirconium  | 0.05-0.10 |

the balance of the alloy being essentially nickel, the total of the molybdenum and tantalum being from 9.75% to 11.25% and the total of the aluminum and titanium being 6.55% to 7.45%.

6. A corrosion resistant nickel-base alloy for use at relatively high temperatures consisting essentially of the following elements in the weight percentages set forth:

|            | Percent |
|------------|---------|
| Chromium   | 8.2     |
| Molybdenum | 6.0     |
| Tantalum   | 4.0     |
| Cobalt     | 10.0    |
| Titanium   | 1.0     |
| Aluminum   | 6.0     |
| Carbon     | 0.1     |
| Boron      | 0.012   |
| Zirconium  | 0.08    |

and the balance of the alloy being essentially nickel.

7. A corrosion resistant nickel-base alloy for use at relatively high temperatures consisting essentially of the following elements in the weight percentages set forth:

|            | Percent |
|------------|---------|
| Chromium   | 8.0     |
| Molybdenum | 4.0     |
| Tantalum   | 8.0     |
| Cobalt     | 14.0    |
| Titanium   | 1.0     |
| Aluminum   | 6.0     |
| Carbon     | 0.1     |
| Boron      | 0.012   |
| Zirconium  | 0.09    |

and the balance of the alloy being essentially nickel.

8. A corrosion resistant nickel-base alloy for use at relatively high temperatures consisting essentially of the following elements in the weight percentages set forth:

|            | Percent |
|------------|---------|
| Chromium   | 8.0     |
| Molybdenum | 8.0     |
| Tantalum   | 4.1     |
| Cobalt     | 10.1    |
| Titanium   | 1.0     |
| Aluminum   | 5.8     |
| Carbon     | 0.08    |
| Boron      | 0.024   |
| Zirconium  | 0.06    |

and the balance of the alloy being essentially nickel.

9. A corrosion resistant nickel-base alloy for use at relatively high temperatures consisting essentially of the following elements in the weight percentages set forth:

|            | Percent |
|------------|---------|
| Chromium   | 7.9     |
| Molybdenum | 3.95    |
| Tantalum   | 7.5     |
| Cobalt     | 9.9     |
| Titanium   | 1.0     |
| Aluminum   | 5.9     |
| Carbon     | 0.1     |
| Boron      | 0.012   |
| Zirconium  | 0.09    |

and the balance of the alloy being essentially nickel.

#### References Cited by the Examiner

##### UNITED STATES PATENTS

|           |         |                 |        |
|-----------|---------|-----------------|--------|
| 2,920,956 | 1/1960  | Nisbet et al.   | 75-171 |
| 3,085,005 | 4/1963  | Michael et al.  | 75-171 |
| 3,107,167 | 10/1963 | Abkowitz et al. | 75-171 |
| 3,202,552 | 8/1965  | Thexton         | 75-171 |

DAVID L. RECK, Primary Examiner.

HYLAND BIZOT, Examiner.

R. O. DEAN, Assistant Examiner.